

## UNITED STATES PATENT OFFICE

2,050,196

PREVENTION OF DETERIORATION OF  
COTTON CORD BY HEATLorin B. Sebrell, Silver Lake, Ohio, assignor to  
Wingfoot Corporation, Wilmington, Del., a  
corporation of DelawareNo Drawing. Application March 1, 1932,  
Serial No. 596,146

14 Claims. (Cl. 8—20)

My invention relates to the treatment of cotton cord to enhance its tensile strength and to enable it to maintain the same at temperatures of the order of those encountered in pneumatic tires under service conditions. The invention includes the process of treating cords and the treated cords.

It has been observed heretofore that cords and threads, especially those prepared from cotton fibers, exhibit under X-rays a definite pattern associated with the molecular structure of the cotton. When subjected to relatively high temperatures, for example, 250 degrees F., a molecular rearrangement occurs which causes the pattern to disappear, such rearrangement being accompanied by premature loss of strength and resultant failure of the cord or thread upon the application of relatively small tensional forces. Upon cooling, the major portion of the original strength is regained.

This loss of strength at relatively high temperatures is particularly objectionable in cords employed in the construction of pneumatic tires, because much heat is developed in the latter when run at high speeds. In truck and bus tires, the temperatures sometimes reach values in excess of 250 degrees F. As a result, the cords of which the tire carcasses are composed and which normally are the principal tension resisting elements in the tire are so weakened that premature ruptures or blowouts tend to occur.

My invention resides in the discovery that ordinary cotton cords, threads, filaments, etc., when treated with reagents of the type herein described, continue to produce a definite X-ray

pattern at temperatures materially above that at which the pattern normally vanishes. Such treated cords possess substantially greater tensile strength at ordinary temperatures and retain their original tensile strength when subjected to relatively high temperatures materially better than ordinary untreated cord. Although numerous reagents have been found more or less effective in retarding or resisting the action of relatively high temperatures in cords, I have established experimentally that certain organic compounds, particularly the amines, are especially satisfactory in this respect.

The following are some of the amines which I have found to be suitable for the purposes mentioned.

|                                     |    |  |  |  |
|-------------------------------------|----|--|--|--|
| Aniline                             |    |  |  |  |
| 2-4-diamino diphenyl amine          |    |  |  |  |
| o-toluidine                         |    |  |  |  |
| Di-methyl $\alpha$ -naphthylamine   | 20 |  |  |  |
| Cyclo hexyl amine                   |    |  |  |  |
| $\alpha$ and $\beta$ -naphthylamine |    |  |  |  |
| 4-amino m-xylene                    |    |  |  |  |
| m-tolylene diamine                  | 25 |  |  |  |
| Di-n-propylamine                    |    |  |  |  |
| Di-iso-amyl amine                   |    |  |  |  |
| Thio phenyl $\beta$ -naphthylamine  |    |  |  |  |
| Di-butyl amine                      |    |  |  |  |
| Piperidine                          |    |  |  |  |
| Di-ethyl amine                      | 30 |  |  |  |
| Allyl amine                         |    |  |  |  |
| Butyl amine                         |    |  |  |  |

The results obtained with these compounds are summarized in the following table:

|    | Chemical                                        | Chemical treatment                                                                                             | Tensiles of treated cord |        | Tensiles of raw cord |        | 40 |
|----|-------------------------------------------------|----------------------------------------------------------------------------------------------------------------|--------------------------|--------|----------------------|--------|----|
|    |                                                 |                                                                                                                | 250° F.                  | 75° F. | 250° F.              | 75° F. |    |
| 40 | Aniline.....                                    | (a) 3 hrs. in aniline at 120° C.....                                                                           | 12.7                     | 19.0   | 10.1                 | 17.2   |    |
|    |                                                 | (b) 3 hrs. in aniline at 120° C., drained, 3 hrs. in CS <sub>2</sub> at 25° C.....                             | 12.7                     | 19.0   | 10.1                 | 17.2   |    |
|    |                                                 | (c) 3 hrs. in aniline at 120° C., drained, 3 hrs. in 30% formaldehyde at 90° C.....                            | 11.9                     | 19.1   | 10.1                 | 17.2   |    |
|    |                                                 | (d) Heated in aniline to 110-120° C., allowed to stand 16 hrs. in liquid, washed in ether.....                 | 12.7                     | 20.4   | 10.4                 | 17.1   | 45 |
| 45 | 2-4-diamino diphenyl amine,<br>o-toluidine..... | 2-4-diamino diphenyl amine under 600 lbs. pressure.                                                            | 11.3                     | 17.5   | 10.1                 | 17.2   |    |
|    |                                                 | Heated in o-toluidine to as near 110-120° C. as possible, allowed to stand 16 hrs. in liquid, washed in ether. | 13.0                     | 20.5   | 10.4                 | 17.1   |    |
| 50 | Di-methyl $\alpha$ -naphthylamine.....          | 2 $\frac{1}{4}$ hrs. in di-methyl $\alpha$ -naphthylamine at 70° C., allowed to stand in solution over night.  | 11.8                     | 18.6   | 10.4                 | 17.1   | 50 |
|    |                                                 | (a) 3 hrs. in cyclo hexyl amine at 76° C.....                                                                  | 13.3                     | 21.0   | 10.4                 | 17.1   |    |
|    |                                                 | (b) 3 hrs. in cyclo hexyl amine at 242° F.....                                                                 | 12.8                     | 20.8   |                      |        |    |

| 5  | Chemical                             | Chemical treatment                                                                                                                                                                                                                                                                                                                                                                                                                                                                                                                                                                                                                                                                                                                                                                   | Tensiles of treated cord |        | Tensiles of raw cord |        | 5  |
|----|--------------------------------------|--------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|--------------------------|--------|----------------------|--------|----|
|    |                                      |                                                                                                                                                                                                                                                                                                                                                                                                                                                                                                                                                                                                                                                                                                                                                                                      | 250° F.                  | 75° F. | 250° F.              | 75° F. |    |
|    | $\beta$ -naphthyl-amine.....         | Heated 50 gms. $\beta$ -naphthylamine in 350 cc. xylene and 25 cc. $C_6H_6$ to as near 110-120° C. as possible, allowed to stand 15 hrs. in liquid, washed in ether.                                                                                                                                                                                                                                                                                                                                                                                                                                                                                                                                                                                                                 | 12.5                     | 20.2   | 10.4                 | 17.1   |    |
| 10 | m-toluylene diamine.....             | Heated 50 gms. m-toluylene diamine in 75 cc. xylene and 350 cc. toluene to as near 110-120° C. as possible, allowed to stand 15½ hrs., washed in ether.                                                                                                                                                                                                                                                                                                                                                                                                                                                                                                                                                                                                                              | 13.2                     | 20.7   | 10.4                 | 17.1   | 10 |
| 15 | Di-n-propyl amine.....               | 2½ hrs. in di-n-propyl amine at 70° C., allowed to stand in liquid over night.                                                                                                                                                                                                                                                                                                                                                                                                                                                                                                                                                                                                                                                                                                       | 12.6                     | 20.1   | 10.4                 | 17.1   | 15 |
|    | Di-iso-amyl amine.....               | 2½ hrs. in di-iso-amyl amine at 70° C., allowed to stand in liquid over night.                                                                                                                                                                                                                                                                                                                                                                                                                                                                                                                                                                                                                                                                                                       | 12.6                     | 19.6   | 10.4                 | 17.1   |    |
|    | Thio phenyl $\beta$ -naphthyl amine. | 22 hrs. in thio phenyl $\beta$ -naphthylamine in benzol at room temperature.                                                                                                                                                                                                                                                                                                                                                                                                                                                                                                                                                                                                                                                                                                         | 11.2                     | 18.0   | 10.7                 | 17.5   |    |
| 20 | Di-butyl amine.....                  | (a) 2 hrs. in 100% dibutyl amine at 220° F., 2 hrs. in crotonaldehyde at 240° F.<br>(b) 3 hrs. in 100% dibutylamine at 162° F.<br>(c) 3 hrs. in 100% dibutylamine at 240° F.<br>(d) 3 hrs. in 100% dibutylamine at 160° F., 3 hrs. in 10% triethanolamine in water at 210° F.<br>(e) 3 hrs. in 100% dibutylamine at 162° F., 3 hrs. in 10% triethanolamine in water at 202° F.<br>(f) 3 hrs. in 100% dibutylamine at 160° F., 3 hrs. in 10% triethanolamine in water at 204° F.<br>(g) 3 hrs. in 100% dibutylamine at 162° F., 3 hrs. in 10% triethanolamine in water at 204° F.<br>(h) 3 hrs. in 100% dibutylamine at 198° F., 1½ hrs. in 20% furfuraldehyde in alcohol at 174° F.<br>(i) 3 hrs. in 100% dibutylamine at 198° F., 1½ hrs. in 20% heptaldehyde in alcohol at 174° F. | 10.7                     | 17.5   | 10.5                 | 18.1   | 20 |
| 25 |                                      | (j) 3 hrs. in 100% dibutylamine at 162° F., 3 hrs. in 10% triethanolamine in water at 204° F.<br>(k) 3 hrs. in 100% dibutylamine at 218° F., 3 hrs. in 20% crotonaldehyde in alcohol at 172° F.                                                                                                                                                                                                                                                                                                                                                                                                                                                                                                                                                                                      | 10.7                     | 20.3   | 10.5                 | 18.1   | 25 |
| 30 |                                      | (l) 3 hrs. in 100% dibutylamine at 162° F., 3 hrs. in 20% triethanolamine in water at 204° F.<br>(m) 3 hrs. in 100% dibutylamine at 198° F., 1½ hrs. in 20% furfuraldehyde in alcohol at 174° F.<br>(n) 3 hrs. in 100% dibutylamine at 198° F., 1½ hrs. in 20% heptaldehyde in alcohol at 174° F.                                                                                                                                                                                                                                                                                                                                                                                                                                                                                    | 10.7                     | 19.0   | 10.5                 | 18.1   | 30 |
| 35 | Piperidine.....                      | (o) 3 hrs. in 100% dibutylamine at 218° F.<br>(p) 3 hrs. in 100% dibutylamine at 218° F., 3 hrs. in 20% crotonaldehyde in alcohol at 172° F.<br>(q) 2½ hrs. in piperidine at 75° C., allowed to stand in liquid over night.                                                                                                                                                                                                                                                                                                                                                                                                                                                                                                                                                          | 12.0                     | 20.4   | 10.4                 | 17.1   | 35 |
| 40 |                                      | (r) 3 hrs. in 100% piperidine at 212° F., 1½ hrs. in 20% furfuraldehyde in alcohol at 174° F.<br>(s) 3 hrs. in 100% piperidine at 212° F., 3 hrs. in 20% heptaldehyde in alcohol at 174° F.<br>(t) 3 hrs. in 100% piperidine at 212° F., 3 hrs. in 20% diethylamine in water at room temperature.                                                                                                                                                                                                                                                                                                                                                                                                                                                                                    | 12.1                     | 20.4   | 10.8                 | -----  | 40 |
| 45 | Diethylamine.....                    | (u) 3 hrs. in 21% diethylamine in water at room temperature.<br>(v) 3 hrs. in 21% diethylamine in water at 75° C.<br>(w) 3 hrs. in 85% diethylamine in water at 65° C.<br>(x) Cord exhausted under vacuum of water pump, 85% diethylamine admitted heated to boiling, 3 hrs. at 65° C.<br>(y) 3 hrs. in 85% diethylamine at 65° C., 3 hrs. in 30% formaldehyde at 90° C.                                                                                                                                                                                                                                                                                                                                                                                                             | 11.7                     | 17.3   | 10.1                 | 17.2   | 45 |
| 50 | Allyl amine.....                     | 2½ hrs. in allyl amine at 70° C., allowed to stand in liquid over night.                                                                                                                                                                                                                                                                                                                                                                                                                                                                                                                                                                                                                                                                                                             | 14.1                     | 20.2   | 10.4                 | 17.1   | 50 |
| 55 | Butyl amine.....                     | (z) 6 hrs. in 50% butylamine in water at 160° F.<br>(a) 3 hrs. in 100% butylamine at 158° F.<br>(b) 3 hrs. in 100% butylamine at 162° F.<br>(c) 72 hrs. in 100% butylamine at 72° F.<br>(d) 3 hrs. in 100% butylamine at 170° F., washed in water.<br>(e) 15 mins. in 15% butylamine in water at 120° F.                                                                                                                                                                                                                                                                                                                                                                                                                                                                             | 10.7                     | 18.5   | 10.7                 | 17.5   | 55 |
| 60 |                                      | (f) 15 mins. in 15% butylamine in water at 120° F.                                                                                                                                                                                                                                                                                                                                                                                                                                                                                                                                                                                                                                                                                                                                   | 11.5                     | 18.6   | 10.7                 | 17.5   |    |
|    |                                      |                                                                                                                                                                                                                                                                                                                                                                                                                                                                                                                                                                                                                                                                                                                                                                                      | 11.5                     | -----  | 10.7                 | 17.5   |    |
|    |                                      |                                                                                                                                                                                                                                                                                                                                                                                                                                                                                                                                                                                                                                                                                                                                                                                      | 12.3                     | -----  | 10.5                 | 18.1   |    |
|    |                                      |                                                                                                                                                                                                                                                                                                                                                                                                                                                                                                                                                                                                                                                                                                                                                                                      | 11.9                     | -----  | 10.7                 | 17.5   |    |
|    |                                      |                                                                                                                                                                                                                                                                                                                                                                                                                                                                                                                                                                                                                                                                                                                                                                                      | 10.6                     | 18.0   | 10.7                 | 17.5   | 60 |

65 In these tests, samples of cord were treated with these reagents, after which one set of samples was tested for tensile strength at normal or approximately room temperatures and at 34 percent relative humidity. The second set of samples was then subjected to tests identical with those conducted upon the first set, except that the temperature was maintained at a value of 250 degrees F. during the test. The control employed was identical in every respect with the treated cord, except that it was not treated.

70 From the table, it will be apparent that cords which have been treated are materially higher in

75 tensile strength both at relatively high temperatures and at ordinary or normal temperatures. In some cases, this increase amounts to as much as 30 to 40 percent at temperatures of 250 degrees. This increase is very advantageous in case the cords are employed in bus tires or similar tires of large size which are run at relatively high speeds.

70 It will be apparent that my invention is not limited to cords employed in pneumatic tires. It may be used in connection with substantially any cotton fabric which is exposed to relatively high temperatures, one particular application being

in connection with fabric employed in the manufacture of hose used to convey heated liquids. It is also to be understood that the invention is not limited to the specific compounds disclosed herein. All amines tested have been found to be effective to some extent, from which it appears probable that all of the compounds of this class exhibit properties of the kind described.

This application is a continuation in part of my prior application Serial No. 420,638, filed January 13, 1930, for Prevention of deterioration of cotton cord by heat, now abandoned.

Although I have described only the preferred forms which the invention may assume, it will be apparent to those skilled in the art that it is not limited thereto, but that various modifications may be made without departing from the spirit of the invention or from the scope of the appended claims. It is intended that the patent shall cover, by suitable expression in the appended claims, whatever features of patentable novelty reside in the invention.

What I claim is:

1. The method of treating cotton which comprises subjecting it to the action of an amine having at least one univalent organic radical attached to the nitrogen atom of the amine as a substituent whereby, without producing any material change in the appearance of the cotton or the way it feels, it is made to have greater tensile strength at 250° F. than untreated cotton at the same temperature.

2. The method of treating cotton which comprises subjecting it at an elevated temperature to the action of an amine selected from the following group:

|                                         |  |
|-----------------------------------------|--|
| Aniline                                 |  |
| 2-4-diamino diphenyl amine              |  |
| o-toluidine                             |  |
| Di-methyl $\alpha$ -naphthyl amine      |  |
| Cyclo hexyl amine                       |  |
| $\alpha$ - and $\beta$ -naphthyl amines |  |
| 4-amino m-xylylene                      |  |
| m-toluylene diamine                     |  |
| Di-n-propylamine                        |  |
| Di-iso-amyl amine                       |  |
| Di-butyl amine                          |  |
| Di-ethyl amine                          |  |
| Allyl amine                             |  |
| Butyl amine                             |  |
| Thio phenyl $\beta$ -naphthyl amine     |  |

whereby, without producing any material change in its appearance or the way it feels, it is made to have greater tensile strength at 250° F. than untreated cotton at the same temperature.

3. The method of treating a cotton cord which comprises subjecting it to the action of a primary amine whereby without producing any material change in its appearance or the way it feels the cord is made to have greater tensile strength at 250° F. than the untreated cord at the same temperature.

4. The method of treating a cotton cord which comprises subjecting it to the action of an aliphatic amine whereby without producing any material change in its appearance or the way it feels the cord is made to have greater tensile

strength at 250° F. than the untreated cord at the same temperature.

5. The method of treating a cotton cord which comprises subjecting it to the action of an aliphatic amine whereby without producing any material change in its appearance or the way it feels the cord is made to have greater tensile strength at 250° F. than the untreated cord at the same temperature.

6. The method of treating a cotton cord which comprises subjecting it to the action of cyclohexyl amine whereby without producing any material change in its appearance or the way it feels the cord is made to have greater tensile strength at 250° F. than the untreated cord at the same temperature.

7. The method of treating a cotton cord which comprises subjecting it to the action of a primary aliphatic amine whereby without producing any material change in its appearance or the way it feels the cord is made to have greater tensile strength at 250° F. than the untreated cord at the same temperature.

8. The method of treating a cotton cord which comprises subjecting it to the action of a butyl amine whereby without producing any material change in its appearance or the way it feels the cord is made to have greater tensile strength at 250° F. than the untreated cord at the same temperature.

9. The method of treating a cotton cord which comprises subjecting it to the action of di-butyl amine whereby without producing any material change in its appearance or the way it feels the cord is made to have greater tensile strength at 250° F. than the untreated cord at the same temperature.

10. The method of treating a cotton cord which comprises subjecting it to the action of aniline whereby without producing any material change in its appearance or the way it feels the cord is made to have greater tensile strength at 250° F. than the untreated cord at the same temperature.

11. A cotton cord treated with an amine, which treated cord has the same general appearance and feels substantially the same as an untreated cotton cord and has greater tensile strength at 250° F. than the untreated cord at the same temperature.

12. A cotton cord treated with aniline, which treated cord has the same general appearance and feels substantially the same as an untreated cotton cord and has greater tensile strength at 250° F. than the untreated cord at the same temperature.

13. A cotton cord treated with a butyl amine, which treated cord has the same general appearance and feels substantially the same as an untreated cotton cord and has greater tensile strength at 250° F. than the untreated cord at the same temperature.

14. A cotton cord treated with cyclohexyl amine, which treated cord has the same general appearance and feels substantially the same as an untreated cotton cord and possesses greater tensile strength at 250° F. than the untreated cord at the same temperature.

LORIN B. SEBRELL.